

1

3,783,014

## ELECTROLESS COATING OF MOYBDENUM ON STAINLESS STEELS

John W. Koger, Knoxville, and Eugene J. Lawrence, Alcoa, Tenn., assignors to the United States of America as represented by the United States Atomic Energy Commission

No Drawing. Filed Jan. 18, 1972, Ser. No. 218,817  
Int. Cl. C23c 9/10, 17/02

U.S. Cl. 117—130 R

2 Claims

### ABSTRACT OF THE DISCLOSURE

An adherent coating of molybdenum on stainless steel is obtained by contacting the stainless steel with a molten fluoride salt containing from 1 to 5 weight percent  $MoF_6$ .

### BACKGROUND OF THE INVENTION

The invention described herein was made in the course of, or under, a contract with the U.S. Atomic Energy Commission.

The present invention relates to a method for depositing a coherent, adherent coating of molybdenum on a stainless steel substrate and to a composition for practicing the method.

The prior art known to the applicants for coating stainless steels with molybdenum consists of electrolytic plating and chemical vapor deposition processes. Both techniques are effective for depositing molybdenum, but are of limited utility in applying a uniform coating to a surface of complex geometry such as the internal surfaces of a piping arrangement or a vessel with relatively inaccessible surface area. In electrolytic processes it is difficult to attain uniform throwing power, and the composition of the electrolytic bath as well as electroplating process parameters must be constantly monitored. Molybdenum cannot be satisfactorily deposited directly upon a stainless steel surface but requires an initial application of a nickel coating to insure good adhesion of molybdenum.

### SUMMARY OF THE INVENTION

The present invention is not subject to the limitations of electroplating or chemical vapor deposition. It comprises, in its process aspect, formulating a molten fluoride salt solvent phase containing from 1 to about 5 weight percent molybdenum fluoride, based on the weight of the solvent phase, and contacting the resultant molybdenum-containing molten salt composition with an iron-, nickel-, or chromium-containing substrate for a time sufficient to effect deposition of molybdenum by a replacement chemical reaction. The molten fluoride solvent phase may consist of an alkali metal fluoride, an alkaline earth fluoride, or any mixture thereof. Typical solvent salts which can be used to practice this invention are listed below:

| Solvent salt:                              | Liquidus (° C.) |
|--------------------------------------------|-----------------|
| $NaF-LiF-KF$ (11.5-46.5-42.0 mole percent) | 459             |
| $NaF-LiF-BeF_2$ (27-35-38 mole percent)    | 338             |
| $NaF-BeF_2-KF$ (30-65-5 mole percent)      | 435             |
| $NaF-KF-ZrF_4$ (5-52-43 mole percent)      | 425             |
| $KF-NaF-ZrF_4$ (18-36-46 mole percent)     | 450             |
| $LiF-BeF_2$ (69-31 mole percent)           | 505             |

The temperature of deposition ranges from a minimum defined by the melting point of the molybdenum-containing fused salt bath up to as much as several hundred degrees beyond with a practical maximum existing where adverse chemical reaction is found to occur. Temperature is used to control the rate of deposition. The temperature of deposition may vary from as low as 300° C. to as high

2

as 800° C. depending on the melting point of the fused salt solvent and the rate of deposition desired. In most cases, the higher temperature will result in a higher rate of molybdenum deposition.

The fused fluoride bath is simply prepared from any combination of alkali or alkaline earth fluorides. Molybdenum is readily introduced into solution by bubbling a gaseous mixture of  $MoF_6$  and an inert carrier gas into the volume of the fused fluoride salt phase until it is present in solution to at least about 1 weight percent  $MoF_6$ . Lower amounts may be useful in selected circumstances, but for most applications a minimum of 1 percent molybdenum fluoride is preferred.

The exact amount of molybdenum required for a particular application can be approximated from and is a function of the composition of the substrate material in the light of the following apparent mechanism of deposition. The deposition process is visualized as taking place by a replacement chemical reaction between molybdenum as the metal constituents of the substrates according to the formula



where

$M = Fe, Cr, or Ni$ ;  
 $a = \text{substrate constituent}$ ;  
 $s = \text{solution}$ ;  
 $d = \text{deposit}$ ; and  
 $n = \text{valence of } M$ .

This reaction involves the oxidation of Fe, Cr, and Ni to their respective fluorides by the reduction of the molybdenum fluoride. The experimental evidence in support of this mechanism is based on analysis of the fluoride salt phase after molybdenum deposition which shows concentrations of Fe, Cr, and Ni in solution at levels comparable to the amount of molybdenum deposited on the metal surface.

To insure continuous adherent coating of molybdenum, the conditions must be controlled such that the substrate fluorides do not exceed their solubility in the molten fluoride composition. Otherwise, the undissolved metal fluorides will codeposit with molybdenum to produce a non-uniform deposit. Solubility can be maintained by temperature and by controlling the amount of molybdenum in solution. At constant temperature, the main controlling variable is the concentration of molybdenum. For most applications, the maximum concentration of molybdenum fluoride in the salt phase should not exceed 5 weight percent in order to avoid exceeding solubility limits of the substrate metal fluorides.

### DESCRIPTION OF A REPRESENTATIVE EMBODIMENT

A sample of Type 316 stainless steel consisting essentially of 17 weight percent Cr, 12 weight percent Ni, 2 weight percent Mo, and the balance Fe was coated with molybdenum according to the following procedure.

Three separate volumes of a molten fluoride salt consisting essentially of  $LiF$  and  $BeF_2$  (about 2:1 mole percent) were heated to 675° C. A gaseous mixture of  $MoF_6$  in a helium carrier was then bubbled through each of the melts until concentrations of 1, 4, and 10 weight percent  $MoF_6$  were established in the respective melts. Sample coupons of Type 316 stainless steel were then immersed in each of the molybdenum-containing melts for a period ranging from 50 to 70 hours at melt temperatures ranging from 650° to 675° C. The coupons were removed and found to have been coated with molybdenum. An adherent and uniform coating of molybdenum was obtained from the melts containing 1 and 4 weight percent molybdenum fluoride. Microprobe analyses indicated that the molybdenum had diffused into the substrate to a depth of

at least 350 microns. While the sample immersed in the bath containing 10 weight percent molybdenum had a continuous coating, some areas were found to be easily removed. Metallographic and microprobe analysis of the samples showed a multilayered coating containing fluorides of lithium, beryllium, iron, and chromium. In this case, the solubility limits of the fluorides of these elements had been exceeded, causing co-deposition of this corrosion product with the molybdenum. Thus it is these fluorides which appeared to be largely responsible for the non-adherence of the molybdenum.

It will be seen that a general method has been described for depositing a uniform adherent deposit of molybdenum on a metal substrate. The method is simple and uncomplicated, and has unique capability in applying a uniform and adherent molybdenum coating on remote surfaces and articles of complicated geometry. A singularly apt application of this process is found in the preparation of apparatus for the chemical processing of spent molten fluoride nuclear fuel compositions involving selective extraction of metal values in the fluoride phase into a liquid bismuth phase. A molybdenum-surfaced container system is needed to withstand the corrosive effects of both molten fluorides and liquid bismuth. With the molybdenum coating process of this invention at hand, it is now possible to construct an entire container system together with associated piping from stainless steel and then simply fill the system at the desired temperature with the molybdenum-containing fused fluoride composition to achieve a uniform adherent coating throughout the sys-

tem. Circulation of the salt through the system will coat all vessels and interconnected piping in the system.

What is claimed is:

1. A method for electrolessly applying an adherent coating of molybdenum on a stainless steel substrate which comprises contacting said substrate with a fused salt comprising at least one alkali metal fluoride, alkaline earth metal fluoride, or mixtures thereof and from 1 to 5 weight percent molybdenum, as  $\text{MoF}_6$ , dissolved in said salt at a temperature and for a period of time sufficient to coat said substrate.

2. The method of claim 1 wherein the temperature of deposition is in the range 300° to 800° C.

#### References Cited

##### UNITED STATES PATENTS

|           |        |                  |             |
|-----------|--------|------------------|-------------|
| 3,444,058 | 5/1969 | Mellors et al.   | 204—39 X    |
| 2,734,003 | 2/1956 | Alpert           | 117—130 R   |
| 2,746,888 | 5/1956 | Ross             | 117—113 X   |
| 2,786,809 | 3/1957 | Raynes           | 204—39      |
| 2,828,251 | 3/1958 | Sibert et al.    | 204—39      |
| 2,872,348 | 2/1959 | Eubank           | 117—130 R X |
| 2,950,233 | 8/1960 | Steinberg et al. | 204—39 X    |
| 3,203,811 | 8/1965 | Boller           | 117—130 R X |

ALFRED L. LEAVITT, Primary Examiner

J. R. BATTEEN, JR., Assistant Examiner

U.S. CL. X.R.

30 106—1, 286; 117—113